

1

3,169,870

**PHOTOGRAPHIC GELATIN LAYERS CONTAINING THE SALTS OF VARIOUS ALKYL AND ALKENYL SUCCINAMATES AS COATING AIDS**

William J. Knox, Jr., Rochester, N.Y., and Robert E. Sticker, Lawrence, Kans., assignors to Eastman Kodak Company, Rochester, N.Y., a corporation of New Jersey

No Drawing. Filed Dec. 4, 1961, Ser. No. 156,976

3 Claims. (Cl. 96—94)

This invention relates to improved gelatin coating compositions containing certain succinamates as coating aids and their application to film base and paper.

In the photographic industry it is frequently desirable to apply two or more gelatin layers to film base or paper. This may be conveniently accomplished by successive coating or by multiple coating as described in U.S. Patent 2,761,791. That patent discloses a method of applying a plurality of separate coatings to the surface of a moving web simultaneously while still maintaining a distinct layer relationship between the coatings after deposition. Essentially, this method involves continuously forming each fluid composition into a layer of given thickness, bringing these layers into surface contact prior to the time they are applied to the surface of the web and directing them while in combined relation to the point of where they are applied simultaneously to the web in the desired orientation with no noticeable mixing or contamination at the interface of the layers. Apparatus for the simultaneous application of multiple coatings is described in U.S. Patents 2,761,417 and 2,761,418. The term "successive coating" refers to coating a gelatin layer on a support and, before that coating has dried, applying another gelatin layer thereover. This method of coating a plurality of gelatin layers on a support is also referred to as "wet-on-wet" coating.

Gelatin coatings applied simultaneously in accordance with the method described in the above-identified patent but without the use of a coating aid, are unsatisfactory in several respects. Crescent-shaped uncoated areas (repellencies) probably attributable to oil impurities in the gelatin are found in the coating. These defects may be about the size of a pinhead with streaks running down from the points of the crescent in a direction opposite to that of the coating. In addition, longitudinal pencil-line streaks and double-edge comets may appear in the coating. Accordingly, a number of coating aids have been tested, some of which have been found to produce blemish-free coatings. However, the coatings produced with these coating aids when dried have been generally considered unsatisfactory because of surface slickness or inadequate rewettability. Handling problems result from surface slickness while inadequate rewettability causes processing difficulties.

A number of coating aids have been suggested to facilitate single-layer gelatin coatings. A notable example is saponin which, when employed in single-layer coatings, effectively suppresses repellencies and yields dried coatings with satisfactory developer wettability and adequate surface roughness. However, in the simultaneous application of two or more gelatin layers to a base or paper, saponin is ineffective to prevent pencil-line streaks and double-edged comets. Saponin is a naturally occurring substance which varies in quality and composition from

2

batch to batch which may cause an increase in fog or a change in photographic sensitivity. Hence, various synthetic coating aids have been proposed for single-layer coatings. A number of synthetic coating aids useful for single-layer coatings have been considered for simultaneous coating operations, but the coatings thus produced are generally unsatisfactory due to surface slickness, inadequate rewettability or defects in the coating itself, such as pencil-line streaks or double-edged comets.

We have now found a class of compounds which may be employed as coating aids in single-layer gelatin coatings, or simultaneous gelatin coating operations to produce blemish-free coatings which, when dried, possess the necessary surface roughness and rewettability.

One object of our invention is to provide improved gelatin coating compositions containing certain succinamates as coating aids. Another object of our invention is to provide a plurality of coating compositions which may be simultaneously applied to a base or paper to produce substantially blemish-free coatings having adequate surface roughness and rewettability. Still other objects of our invention will appear herein.

We have now found that by incorporating certain succinamates as coating aids in gelatin coating compositions, improved single-layer coatings are obtained. We have also found that these succinamates may be incorporated into a plurality of gelatin coating compositions which may be coated successively or simultaneously onto film base or paper. The succinamates which we have found to be useful are indicated in the following formula:



35 one of  $\text{R}_1$  and  $\text{R}_2$  being H, the other being selected from the group consisting of alkyl and alkenyl radicals containing 8-16 carbon atoms having at least two points of branching;  $\text{R}_3$  is selected from the group consisting of H,  $-\text{CH}_3$ ,  $-\text{CH}_2\text{CH}_2\text{OH}$  and  $-\text{CH}_2\text{CH}_2\text{CH}_2\text{OH}$ ;  $\text{R}_4$ , where  $\text{R}_3$  is selected from the group consisting of H and  $-\text{CH}_3$ , is selected from the grouping consisting of



40 (x being 2-5 and y being 1-4, the sum of x and y being 3-9) and  $-\text{C}(\text{CHOH})_2(\text{CH}_2)_n\text{CH}_3$  (n being 0 to 3),  $\text{R}_4$ , where  $\text{R}_3$  is selected from the group consisting of  $-\text{CH}_2\text{CH}_2\text{OH}$  and  $-\text{CH}_2\text{CH}_2\text{CH}_2\text{OH}$ , is selected from the group consisting of  $-\text{CH}_2\text{CH}_2\text{OH}$ ,



45 and the alkyl radicals containing 2 to 5 carbon atoms and, M is a salt forming radical such as Na, K,  $\text{NH}_4$ , mono-, di- or triethanolammonium.

50 It may be seen that generally two isomeric forms of the compounds of our invention are possible. Thus, referring to the generic formula shown above, it is apparent that the branched-chain alkyl or alkenyl radical may be positioned on the succinic radical beta or gamma to the nitrogen atom. It is believed (but not known) that one isomer predominates in the normal preparation of the compounds of this invention. In any event, a mixture of 55 the isomers appears satisfactory in employing the com-

pounds of the invention as coating aids in protein coating compositions.

The compounds of this invention may be prepared by reacting the desired branched-chain alkyl or alkenyl succinic anhydried with the desired amine in the presence of heat and a base such as sodium hydroxide. Particularly valuable coating aids may be prepared by reacting commercially available dodecenylysuccinic anhydride (wherein the dodecetyl radical is a mixture of branched monoolefins formed by tetramerizing propene) with a compound selected from the group consisting of 2,2'-iminodiethanol; N-methylglucamine; and 1-[2-(2'-hydroxy)ethoxy-2-ethoxyethoxy-3-aminopropane]. The structural formulas of the coating aids thus produced are indicated below.

Surfactant "A":



and



Surfactant "C":



and



Surfactant "D":



and



The dodecetyl radical of the above compounds contains not less than two points of branching, and generally is a highly branched monoolefin radical. As indicated above, various other alkyl and alkenyl substituted succinamates may be employed in accordance with this invention. Representative examples include the following: a tetramethylbutylsuccinamic acid, sodium salt; a branched-chain dodecylsuccinamic acid, sodium salt; a branched-chain tridecylsuccinamic acid, sodium salt; a branched-chain pentadecylsuccinamic acid, sodium salt; a branched-chain hexadecylsuccinamic acid, sodium salt; a branched-chain nonenylsuccinamic acid, sodium salt; a branched-chain dodecylsuccinamic acid, sodium salt; a branched-chain pentadecylsuccinamic acid, sodium salt; and, a branched-chain hexadecylsuccinamic acid, sodium salt. In each of the foregoing compounds, the alkyl or alkenyl radical contains not less than two points of branching. Of course, the substituents attached to the nitrogen atom in these compounds conform to the general description of the succinamates of our invention given above.

The coating materials containing our agent may be of various compositions. However, for general explanation, reference will be made to proteinaceous coating compositions of a photographic nature. Such coatings are illustrated by gelatin containing various sensitive components such as silver salts. This type of composition is referred to in some detail inasmuch as it concerns our preferred embodiment and also presents more problems than certain other coating compositions. That is, while in the art many kinds of surface-active agents have been added to coating compositions and do facilitate their coating, nevertheless such agents would not be suitable in compositions such as the photographic coatings under description since such agents may injure the light-sensitive photographic

materials. Hence, it is thought that by showing that the present invention functions in an environment of light-sensitive photographic coatings, it will be apparent that even where the problem of photographic sensitivity is not present, our invention would likewise have utility and application.

As just mentioned, photographic coatings are comprised of a medium such as gelatin which contains light-sensitive material comprising a silver salt such as silver chloride or bromide. The emulsion may likewise contain dyes and various other materials. Inasmuch as a description of emulsion coatings is found in the publication "Fundamentals of Photographic Theory" by T. H. James and George C. Higgins, published in 1948 by John W. Wiley & Sons, Inc., Chapter 2, further detailed description herein appears unnecessary.

The base to be coated may be composed of any of the usual conventional base materials. In this invention particular reference is made to a paper base. A description 20 of photographic paper is found in Kodak Data Book, 5th Edition, "Kodak Papers," pages 3 and 4. A base material of this type would preferably be used in the present invention.

The over-all coating procedures which may be utilized 25 comprise any of the standard procedures employed in the industry. Chief among these are the extrusion hopper coatings from which the coating melt in a single layer coating is delivered at a measured rate, or various coating melts in a multilayer coating are delivered simultaneously, 30 each at a measured rate, to the support so as to give dried coatings with layers of the desired thickness in accordance with the method outlined in U.S. Patent 2,761,791, with apparatus disclosed in U.S. Patent 2,761,417, or 2,761,418.

In practicing our invention, the coating composition 35 which it is desired to apply to a film base or paper is prepared in the usual manner. However, at some time before the actual coating operation there is incorporated into the coating composition a surface-active agent of the present invention. This incorporation may be accomplished advantageously in the following manner: A 2.5% aqueous solution of the coating aid may be prepared. An amount equal to 0.04 to 1.0 gram (dry weight) of coating aid per 454 g. of coating solution is added to the gelatin-silver halide emulsion at any point after the emulsion is 45 in a liquid state, either before, during, or after the addition of other materials.

A further understanding of our invention will be had 50 from a consideration of the several specific examples which follow. In these examples a single pelloid coating was applied to a film base, using the preferred coating aids referred to above at a concentration of 0.22 gram per 454 g. of wet coating melt. The results are shown in the following table:

Table I

|    | Surfactant   | Repellencies<br>on 25 sq. ft.<br>of Coating | Mottle      | Longitudinal<br>Streaks |
|----|--------------|---------------------------------------------|-------------|-------------------------|
| 60 | A-----       | 0                                           | Very Slight | Very Slight             |
|    | C-----       | 0                                           | do          | do                      |
|    | D-----       | 0                                           | do          | do                      |
| 65 | Control----- | 21                                          | Slight      | Slight                  |

In the above table, by "Repellencies" we refer to the number of uncoated spots. The Control involved a similar coating experiment in which no surfactant was used.

A series of experiments were conducted in which a gelatin-silver halide photographic emulsion and its clear gelatin overcoat were applied simultaneously to a paper support using a hopper technique and coating aids in accordance with our invention in each layer. The results 75 are shown in the following table:

Table II

| Surfactant | Concentration of Surfactant, g. |                                | Developer Spread,<br>cm. <sup>2</sup> | Coefficient of Friction <sup>2</sup> | Repel-<br>lencies <sup>3</sup> |
|------------|---------------------------------|--------------------------------|---------------------------------------|--------------------------------------|--------------------------------|
|            | Per 454 g.<br>Emulsion          | Per 454 g.<br>Clear<br>Gelatin |                                       |                                      |                                |
| A          | 0.13                            | 0.5                            | 8.55                                  | 0.497                                | None.                          |
| A          | 0.25                            | 0.5                            | 12.60                                 | 0.497                                | Do.                            |
| A          | 0.5                             | 0.5                            | 15.90                                 | 0.497                                | Do.                            |
| C          | 0.13                            | 0.5                            | 6.60                                  | 0.408                                | None.                          |
| C          | 0.25                            | 0.5                            | 13.90                                 | 0.442                                | Do.                            |
| C          | 0.5                             | 0.5                            | 9.08                                  | 0.408                                | Do.                            |
| D          | 0.13                            | 0.5                            | 8.04                                  | 0.276                                | None.                          |
| D          | 0.25                            | 0.5                            | 9.08                                  | 0.276                                | Do.                            |
| D          | 0.5                             | 0.5                            | 11.90                                 | 0.276                                | Do.                            |

<sup>1</sup> One cc. of developer solution is delivered to a surface of a paper support coated with a photographic emulsion and a clear gelatin coat thereover, and the area which develops in about 30 seconds was measured. This test indicates how effectively an emulsion containing a coating aid of our invention will wet. A developer spread of 4.0 cm.<sup>2</sup> or more is desirable.

desirable.

2 Two sheets of a paper support were coated with a gelatin-silver halide photographic emulsion and a clear gelatin coating thereover, and one sheet was placed upon the other so that the uncoated side of one paper support, was against the coated side of the other paper support. The coefficient of friction was measured to determine the slickness of gelatin coatings containing the coating aids of this invention. Difficulties occur in stacking coated sheets when the coefficient of friction is less than about .25.

<sup>3</sup> The number of uncoated spots on 7.5 sq. ft. of coating.

The occurrence of pencil-line streaks is a persistent defect in coatings achieved by the simultaneous application of two gelatin layers to a film base or paper. The ability of a coating aid to reduce the incidence of pencil-line streaks is indicated when 1 ml. of a 7% photographic gelatin-silver halide emulsion, containing the coating aid, has a spread of at least 5.0 cm.<sup>2</sup> when coated in a standard manner on a soap-cleaned, horizontal surface of a highly polished stainless steel plate. Employing this test, various coating aids of our invention and saponin, were tested in different concentrations, to determine their ability to control pencil-line streaks in simultaneously applied gelatin coatings. The results are shown in Table III.

Table III

| Surfactant Concentration,<br>grams per pound | Surfactant          |                     |                     | Saponin |
|----------------------------------------------|---------------------|---------------------|---------------------|---------|
|                                              | A, cm. <sup>2</sup> | C, cm. <sup>2</sup> | D, cm. <sup>2</sup> |         |
| 0.0                                          | 3.7                 | 3.7                 | 3.8                 | 3.      |
| 0.07                                         | 5.0                 | 5.2                 |                     |         |
| 0.13                                         | 5.0                 | 5.5                 | 6.4                 | 4.      |
| 0.25                                         | 6.7                 | 7.1                 | 7.0                 | 4.      |
| 0.5                                          | 7.1                 | 7.2                 | 7.8                 | 4.      |

Although the invention has been described in considerable detail with reference to certain preferred embodiments thereof, it will be understood that variations and modifications can be effected within the spirit and scope of the invention as described hereinabove and as defined in the appended claims.

We claim:

1. A composition of matter comprising gelatin containing as a coating aid a compound having the following formula:



one of  $R_1$  and  $R_2$  being H, the other being selected from the group consisting of the alkyl and the alkenyl radicals containing 8-16 carbon atoms having at least two points of branching;  $R_3$  is selected from the group consisting of  $-H$ ,  $-CH_3$ ,  $-CH_2CH_2OH$  and  $-CH_2CH_2CH_2OH$ ;  $R_4$ , where  $R_4$  is selected from the group consisting of H

and  $-\text{CH}_3$ , is selected from the group consisting of  $-\text{CH}_2(\text{CHOH})_4\text{CH}_2\text{OH}$ ,

<sup>5</sup> (x being 2-5, y being 1-4, the sum of x and y being 3-9), and  $-\text{C}(\text{CH}_2\text{OH})_2(\text{CH}_2)_n\text{CH}_3$  (n being 0-3); R<sub>4</sub>, where R<sub>3</sub> is selected from the group consisting of  $-\text{CH}_2\text{CH}_2\text{OH}$  and  $-\text{CH}_2\text{CH}_2\text{CH}_2\text{OH}$ , is selected from the group consisting of  $-\text{CH}_2\text{CH}_2\text{OH}$ ,

10  $\text{---CH}_2\text{CH}_2\text{CH}_2\text{OH}$   
 $\text{---CH}_2(\text{CHOH})_4\text{CH}_2\text{OH}$  and the alkyl radicals containing

2 to 5 carbon atoms; and, M is a salt forming substituent.

15 2. A photographic element comprising a flexible photographic base, a light-sensitive coating thereon containing a gelatin silver halide emulsion, and a clear gelatin coating thereover, at least one of the latter two coatings containing as a coating aid a compound having the following formula:



25 one of  $R_1$  and  $R_2$  being  $H$ , the other being selected from the group consisting of the alkyl and the alkenyl radicals containing 8-16 carbon atoms having at least two points of branching;  $R_3$  is selected from the group consisting of  
 30  $-H$ ,  $-CH_3$ ,  $-CH_2CH_2OH$  and  $-CH_2CH_2CH_2OH$ ;  $R_4$ , where  $R_3$  is selected from the group consisting of  $H$  and  $-CH_3$ , is selected from the group consisting of  
 $-CH_2(CHOH)_4CH_2OH$ ,

(x being 2-5, y being 1-4, the sum of x and y being 3-9), and  $-\text{C}(\text{CH}_2\text{OH})_2(\text{CH}_2)_n\text{CH}_3$  (n being 0-3); R<sub>4</sub>, where R<sub>3</sub> is selected from the group consisting of  $-\text{CH}_2\text{CH}_2\text{OH}$  and  $-\text{CH}_2\text{CH}_2\text{CH}_2\text{OH}$ , is selected from the group consisting of  $-\text{CH}_2\text{CH}_2\text{OH}$ ,

40 —CH<sub>2</sub>CH<sub>2</sub>CH<sub>2</sub>OH  
 —CH<sub>2</sub>(CHOH)<sub>4</sub>CH<sub>2</sub>OH and the alkyl radicals containing 2 to 5 carbon atoms; and, M is a salt forming substituent, which coating aid provides the photographic element with good surface roughness to prevent slippage  
 45 when sheets of the photographic element are stacked upon one another, and imparts good rewettability characteristics to facilitate development of the photographic element.

3. A gelatin-silver halide emulsion containing as a coating aid a compound having the following formula:



one of  $R_1$  and  $R_2$  being H, the other being selected from the group consisting of the alkyl and the alkenyl radicals containing 8-16 carbon atoms having at least two points of branching;  $R_3$  is selected from the group consisting

60 of  $-\text{H}$ ,  $-\text{CH}_3$ ,  $-\text{CH}_2\text{CH}_2\text{OH}$  and  $-\text{CH}_2\text{CH}_2\text{CH}_2\text{OH}$ ;  $\text{R}_4$ , where  $\text{R}_3$  is selected from the group consisting of  $\text{H}$  and  $-\text{CH}_3$ , is selected from the group consisting of  $-\text{CH}_2(\text{CHOH})_4\text{CH}_2\text{OH}$ ,

65  $-(CH_2)_x-O-(CH_2CH_2O)_yH$   
 (x being 2-5, y being 1-4, the sum of x and y being 3-9), and  $-C(CH_2OH)_2(CH_2)_nCH_3$  (n being 0-3).  
 R<sub>4</sub>, where R<sub>3</sub> is selected from the group consisting of  
 $-CH_2CH_2OH$  and  $-CH_2CH_2CH_2OH$ , is selected from  
 the group consisting of  $-CH_2CH_2OH$ ,

—CH<sub>2</sub>CH<sub>2</sub>CH<sub>2</sub>OH  
 —CH<sub>2</sub>(CHOH)<sub>4</sub>CH<sub>2</sub>OH and the alkyl radicals containing 2 to 5 carbon atoms; and, M is a salt forming substituent, which photographic emulsion, because of the presence of said coating aid, is capable of being coated as

a single layer and simultaneously with another proteinaceous coating onto a photographic support to provide a dried down layer substantially free from blemishes and having, because of the presence of said coating aid, sufficient surface roughness to prevent slippage when sheets of the photographic element are stacked upon one another, and good rewettability characteristics to facilitate development of said emulsion.

## References Cited in the file of this patent

10

## UNITED STATES PATENTS

|           |             |               |
|-----------|-------------|---------------|
| 2,304,287 | Schur       | Dec. 8, 1942  |
| 2,823,123 | Knox et al. | Feb. 11, 1958 |

|             |
|-------------|
| 2,899,327   |
| 2,933,406   |
| 2,940,854   |
| 2,952,566   |
| 5 3,003,877 |
| 3,026,202   |
| 3,038,804   |
| 3,042,522   |
| 3,068,101   |

|                    |                |
|--------------------|----------------|
| Christopher et al. | Aug. 11, 1959  |
| Salzberg et al.    | Apr. 19, 1960  |
| Gray               | June 14, 1960  |
| Condax             | Sept. 13, 1960 |
| McLaughlin et al.  | Oct. 10, 1961  |
| Knox et al.        | Mar. 20, 1962  |
| Knox et al.        | June 12, 1962  |
| Ben Ezra           | July 3, 1962   |
| Knox et al.        | Dec. 12, 1962  |

## FOREIGN PATENTS

|        |               |
|--------|---------------|
| Russia | July 18, 1959 |
|--------|---------------|